

July 22, 1958

J. K. HUBBARD

2,844,491

PAPER-LIKE PELLICLE AND METHOD FOR PRODUCING SAME

Filed April 29, 1955

*Fig. 1*



*Fig. 2*



INVENTOR

JAMES K. HUBBARD

BY

*Francis H. Dey*  
ATTORNEY

# United States Patent Office

2,844,491

Patented July 22, 1958

1

2,844,491

## PAPER-LIKE PELLICLE AND METHOD FOR PRODUCING SAME

James K. Hubbard, Longview, Wash., assignor to E. I. du Pont de Nemours and Company, Wilmington, Del., a corporation of Delaware

Application April 29, 1955, Serial No. 505,040

6 Claims. (Cl. 117—65)

This invention relates to a new article of manufacture. More particularly it is concerned with paper and paper-like products from nylon fibers.

Despite the inherent desirable properties of the wholly synthetic fibers which have been commercialized in recent years, these fibers have not begun to replace cellulose in the manufacture of paper-like structures. The high wet strength, toughness, chemical durability, excellent dimensional stability and ageing qualities of these fibers, should make them particularly applicable to the field of paper-like products. One factor which has hindered the development of the wholly synthetic fibers in this field is the inability of the fibers to fibrillate and bond to themselves in the manner of beaten cellulose fibers. In addition, in many cases, commercial paper-making techniques either are not applicable or must be expensively modified to accommodate the bonding process.

It is an object of this invention to provide a new paper structure from nylon fibers.

A further object is to provide a nylon paper-like pellicle of high fold endurance.

Another object is to provide a process for the manufacture of nylon fiber paper which is readily adaptable to commercial paper-making equipment.

These and other objects will become apparent in the course of the following specification and claims.

In accordance with the present invention a paper-like pellicle of an unwoven mass of molecularly oriented synthetic condensation polyamide fibers is bonded with an N-alkoxymethyl polyamide resin. Such materials are described in Cairns, United States Patent No. 2,467,186. The bonding of the polyamide fibers is readily accomplished on commercial paper-making equipment by impregnating an unwoven web or waterleaf of the polyamide fibers with an aqueous dispersion of the N-alkoxymethyl polyamide, squeezing to remove the excess liquid, drying the impregnated web and thereafter pressing. The resulting product, while exhibiting the mechanical and chemical properties of polyamides, possesses fold-endurance values in the order of 700,000 to 1,000,000 cycles and higher.

By an "N-alkoxymethyl polyamide resin" is meant a polyamide containing recurring units of the formula:



wherein R is the non-hydroxyl portion of an alcohol, preferably alkyl or hydrocarbon. Such materials and their aqueous dispersions are described in United States Patent No. 2,467,186.

By a polyamide fiber is meant a funicular structure having molecular orientation, such as a fiber, filament, staple and the like produced from a synthetic linear polyamide, e. g. as described in United States Patent No. 2,071,253 and 2,130,948, by the conventional methods. Among the specific polyamides included within the present invention are those formed by the condensation polymerization of a dibasic acid or an amide-forming de-

2

rivative thereof, such as adipic, sebacic, suberic, azelaic acids or the like, and a diamine such as piperazine, bis-amino cyclohexane, ethylene, trimethylene, pentamethylene, hexamethylene, decamethylene, paraxylylene diamines and the like. Such materials may also be formed by other well known methods such as by polymerization of amino acids or caprolactam.

Figure 1 is a diagrammatical sketch of a paper-like pellicle produced in accordance with the present invention.

Figure 2 is a diagrammatical sketch of an enlarged section of the paper-like pellicle of Figure 1.

In Figure 1, the fibrous nature of the pellicle has been emphasized, for in many instances the pellicle has a paper-like finish and the fibers are not apparent.

In Figure 2, the fibers 1 are bonded together by the N-alkoxymethyl polyamide bonding agent 2 of the present invention.

The following examples are cited to illustrate the invention. They are not intended to limit it in any manner.

All test results to which reference is made in the examples are obtained by following the procedures reported in TAPPI Standards. Fold endurance tests are made on an "M. I. T. Folding Endurance Tester" manufactured by the Tinius Olsen Testing Machine Company.

### EXAMPLE I

Four grams of  $\frac{5}{8}$  inch, 3 denier per filament staple of polyhexamethylene adipamide is suspended in a 6-liter aqueous solution containing 3 grams of sodium carboxymethyl cellulose. The suspension is dispersed on a Rice-Barton "Dyno" pulper having two five-inch concave discs countercurrently stirring at 5000 revolutions per minute at opposite ends of a 5 gallon reservoir. Homogeneity is attained after 2 minutes. Thereafter the aqueous dispersion is filtered over an 8" x 8" square of 80 mesh screen, producing a randomly disposed mat of fibers referred to hereinafter as a "waterleaf." A vacuum of 350 mm. is employed to facilitate moisture removal and to avert bubble entrainment. The waterleaf is gently showered with 20 liters of water to wash out residual sodium carboxymethyl cellulose. The dry waterleaf is then dipped in a 20% solids aqueous dispersion of N-methoxymethyl polyhexamethylene adipamide having 45% of its amide groups substituted with methoxymethyl groups. The impregnated sheet is put through squeeze rolls to remove the excess dispersion and dried. It is thereafter pressed for 30 seconds at 160° C. under a pressure of 200 pounds per square inch. The resulting paper-like pellicle, comprising 89% polyamide fibers and 11% by weight of bonding agent has a tensile strength of 35 pounds per inch, a burst strength of 140 pounds per square inch, elongation of 60%, a tear strength of better than 3200 grams and a folding endurance of 777,329 cycles.

Table 1 below is a summary of various other fibrous polyhexamethylene adipamide pellicle preparations illustrating other polymeric dispersions in comparison with the N-alkoxymethyl polyamide dispersion in various concentrations. The fibers, the conditions and the technique of

Example I are employed in each example. They average about 2.5 ounces per square yard. The impregnated sheets average about 5-8 mils in thickness. "Hycar" Acrylic Rubber #1551 is the trademark of B. F. Goodrich Chemical Co. for a colloidal suspension of an oil-resistant butadiene/acrylonitrile copolymer rubber in a water emulsion. "Chemigum" 245AHS is the trademark of Goodyear Tire and Rubber Co. for a colloidal suspension of an oil resistant butadiene/acrylonitrile copolymer rubber in a water emulsion. "Geon" Latex #552 is the trademark of B. F. Goodrich Chemical Co. for a stable water dispersion of a modified polyvinyl chloride resin

plasticized with "Hycar" acrylic rubber. Copolyamide of Example 8 is a low softening plastic type made from hexamethylene diamine, adipic acid, sebacic acid and caprolactam to yield a copolymer of approximately 35% polyhexamethylene adipamide units, 38% epsilon-aminocaproamide units and 27% polyhexamethylene sebacamide units. Polystyrene Emulsion "P" is an aqueous dispersion of plasticized polystyrene produced by Koppers Co., Inc.

or dropped upon a surface, or a continuous filament may be cross-lapped on a surface. The funicular structure may be crimped or uncrimped and of circular or irregular cross section.

Among N-alkoxymethyl polyamides which are suitable in the process of the present invention may be mentioned N-methoxymethyl polyhexamethylenesebacamide, N-isobutoxymethyl polyhexamethyleneadipamide, N-allyloxy-methyl polyhexamethyleneadipamide, the N-benzyloxy-

Table I

| Example | Binder                     | Solids in Dispersion (percent) | Fiber: Binder (Ratio) | Tensile Strength (lbs./in.) | Fold Endurance (Cycles) |
|---------|----------------------------|--------------------------------|-----------------------|-----------------------------|-------------------------|
| 2       | Same as Ex. 1              | 5                              | 1:0.2                 | 33                          | 700,000 to 1,000,000    |
| 3       | Same as Ex. 1              | 10                             | 1:0.7                 | 47                          |                         |
| 4       | Hycar Acrylic Rubber #1551 | 5                              | 1:0.5                 | 7.9                         | 576                     |
| 5       | Chemigum 245 AHS           | 5                              | 1:0.35                | 8.2                         | 1,638                   |
| 6       | Polystyrene Emulsion "P."  | 5                              | 1:0.76                | 14.3                        | 2,486                   |
| 7       | Geon Latex #552            | 5                              | 1:0.23                | 26                          | 15,000                  |
| 8       | Copolyamide                | 5                              | 1:0.34                | 40                          | 175,000                 |

In general the mechanics of the process described herein are analogous to those of paper making. Thus the process is readily adaptable to paper-making equipment, although not limited thereto. In one embodiment a batt of fibers is formed on a moving screen. Since the fiber stock can be added from a liquid suspension, the Fourdrinier machine is convenient for this operation. The N-alkoxymethyl polyamide dispersion, however, should be applied to the batt after its formation on the endless screen. Addition of the polyamide dispersion to the beater or mixer will not produce the outstanding products of this invention. Adequate heat and pressure for completing the bonding of fibers is supplied conveniently by passing the impregnated batt through heated calender rolls. Manufacture may also be performed on the cylinder paper machine by similar modification.

The method employed in forming the batt is not critical. It is not necessary that the molecularly oriented fibers be suspended in a liquid and beaten prior to batt formation since adherence among the fibers does not depend on fibrillation as is the case in cellulose paper manufacture. However, to attain uniform distribution it is convenient to suspend a known weight of fibers or the like in a measured quantity of liquid and agitate. Machines used in paper making such as the Hollander Beater, the Tug-boat Pulper, Jordans and the like are all suitable. To assist dispersion the viscosity of the liquid may be raised. This may be accomplished by supplying an additive to water such as sodium carboxymethyl cellulose, partially hydrolyzed polyvinyl acetate (such as "Elvanol 72-51" manufactured by E. I. du Pont de Nemours and Co. of Wilmington, Delaware), the condensation product of ethanolamine with mixed long chain acids (such as "Ninol 2012A", manufactured by Ninol Laboratories of Chicago, Illinois), or the like, or by employing a high viscosity liquid such as glycerine, ethylene glycol, t-butyl alcohol or the like. The optimum viscosity will vary with the type of mixing or beating, the fiber denier, and similar factors. In choosing the suspending media and thickener, therefore, care must be exercised to avoid substances which cannot be subsequently removed from the formed batt with ease since certain foreign substances such as for instance sodium carboxymethyl cellulose, even in minute concentrations, have been found to interfere with the formation of the join. In batt formation from a liquid suspension the use of staple having a length below about 1 inch with a denier per filament within the range of from about  $\frac{1}{10}$  to about 6 is preferred. However these values may vary. Fibers of mixed length and denier are suitable. Fibers as short as  $\frac{1}{8}$  inch are satisfactory. Instead of laying the batt from liquid suspension, staple, fiber or filament in wet or dry condition may be blown

methyl polyamide derived from a mixture of hexamethylene diammonium adipate and hexamethylenediammonium sebacate, N-furyloxyethylsebacamide, N-(beta-hydroxyethoxy)methyladipamide, and the like.

The aqueous dispersion of the N-alkoxymethyl polyamide bonding agent is applied to preformed batt in any suitable manner. The amount of bonding resin retained by the batt will depend, of course, on the density of the batt, the solids concentration of the dispersion and the method of removing the excess dispersion. Vacuum filtration of the freshly impregnated batt yields the lowest ratio of binder to fiber in the finished product, all other conditions being equal. The simplest method for controlling porosity of the paper-like product is through variation of the solids content of the aqueous dispersion of N-alkoxymethyl polyamide. Binder to fiber ratios of less than 1:1 are generally preferred if a product with any degree of porosity is desired. If the product contains as much binder as fiber, it is film like and has low tear strength. The binder to fiber ratio may be as low as 0.05:1 and provide adequate bonding for many purposes. In general, the ratio will be between 0.2:1 and 0.7:1 for maximum utility. To obtain these ratios, the aqueous dispersion will vary in solids content between 1 and 10%, depending to some extent upon the method of removing the excess dispersion from the impregnated batt.

The bonding step is generally accomplished by exposure of the resin impregnated batt of nylon fibers to elevated temperature and pressure. The optimum temperature will vary with the specific N-alkoxymethyl polyamide used, the pressure upon the batt and the period of exposure. For a contact period of about thirty seconds a temperature within the range of from about 90 to about 170° C. is usually adequate. While longer heating periods when operating within this temperature range may be employed without deleterious effects, short periods of three minutes or less are preferred to facilitate commercial operations. Temperatures sufficient to induce molecular randomization cause a weakening of the product and loss of flexibility. For the production of a high strength, hard surface paper-like pellicle, a pressure within a range of from about 50 to about 500 pounds per square inch is usually employed. A lower pressure (0 to 5 lbs.) produces a bulkier product of softer surface.

The product is a tough, flexible, coherent paper-like pellicle. It is useful in the making of paper money, as a filter media, as a non-woven fabric, in the manufacture of reinforced plastic, as body armor, condenser paper, in high frequency electronic circuits, printed electrical circuits, stencils, permanent ledger, wall-paper, and the like. While the invention has been exemplified in the production of flat structures, it is obvious that shaped

articles may be similarly formed by depositing the batt or leaf over a form and thereafter applying the necessary heat and pressure. The seamless cones, bags, apparel and the like may be made.

Many equivalent modifications within the inventive concept will be apparent to those skilled in the art from a reading of the foregoing description without a departure from the inventive concept.

What is claimed is:

1. A process of preparing a paper-like pellicle which comprises impregnating an unwoven web of a molecularly oriented synthetic condensation polyamide fiber with an aqueous dispersion of an N-alkoxymethylpolyamide and thereafter subjecting the impregnated mass to heat and pressure.

2. The process of claim 1 wherein the polyamide fiber is hexamethylene adipamide.

3. The process of claim 1 wherein the N-alkoxymethylpolyamide is N-methoxymethyl polyhexamethylene adipamide.

4. A paper-like pellicle comprising an unwoven mass of a molecularly oriented synthetic condensation polyamide fiber adhered at points of fiber intersection with N-alkoxymethylpolyamide.

5. The product of claim 4 wherein the fiber is hexamethylene adipamide.

6. The product of claim 4 wherein the N-alkoxymethylpolyamide is N-methoxymethyl polyhexamethylene adipamide.

10

References Cited in the file of this patent

UNITED STATES PATENTS

|           |                  |               |
|-----------|------------------|---------------|
| 2,714,075 | Watson et al.    | July 26, 1955 |
| 2,714,097 | Watson et al.    | July 26, 1955 |
| 2,715,588 | Graham et al.    | Aug. 16, 1955 |
| 2,774,687 | Nottebohm et al. | Dec. 18, 1956 |

OTHER REFERENCES

20 Merriam-Webster's New International Dictionary, 2nd ed. page 2894, item "web."